

## UNITED STATES PATENT OFFICE

2,179,195

## MANUFACTURE OF ARTIFICIAL SILK

James J. Polak, Arnhem, and Johannes G. Weelde-  
enburg, Ede, Netherlands, assignors to Ameri-  
can Enka Corporation, Enka, N. C., a corpora-  
tion of Delaware

No Drawing. Original application January 25,  
1937, Serial No. 122,323. Divided and this ap-  
plication June 6, 1938, Serial No. 212,184. In  
Germany February 15, 1935

10 Claims. (Cl. 18—54)

This application is a division of our applica-  
tion Serial Number 122,323, filed January 25, 1937  
now Patent No. 2,125,031, the latter being a con-  
tinuation in part of our application Serial No.  
51,332, filed November 23, 1935.

The present invention has to do with a new  
and novel method for use in the manufacture of  
yarn or other materials of artificial origin and  
the products thereof.

10 More specifically, the present invention con-  
cerns a novel process for maintaining ideal spin-  
ning conditions in the manufacture of yarn of  
artificial origin.

In the manufacture of artificial filaments,  
15 threads, yarns, ribbons and the like, a cellulosic  
solution is prepared and expressed or extruded  
through minute openings into a coagulating or  
precipitating medium. This medium is usually  
either liquid or gaseous.

20 In preparing the cellulosic spinning solutions  
referred to in the specific examples of the present  
case, cellulose is treated with caustic to form  
alkali cellulose, which, with carbon disulphide,  
25 produces a xanthate. This, in solution, produces  
a viscose spinning solution.

25 In the present specification we shall describe  
our invention with respect to a viscose process,  
but it must be understood that the underlying  
30 principle is broad, and that we do not wish to  
be limited to any specific, minute application of  
our concept.

In the commercial production of artificial yarn  
and analogous products, it is economically neces-  
35 sary, if possible, to provide for uninterrupted  
spinning of all filaments. Ordinarily the objec-  
tions arising which occasion interruptions to the  
spinning or extruding step, are caused by the con-  
tamination of the spinnerets themselves. This  
40 fault can, we believe, be traced to the presence of  
suspensions, reaction products, and impurities of  
various kinds in the viscose solution or the spin-  
ning bath which tend to agglomerate or deposit on  
the spinneret and partially or entirely block the  
45 small orifices therein. These materials might in-  
clude, among others, precipitated cellulose, sul-  
phur deposits, particles of resin, secondary reac-  
tion products, and the like.

We have noted this phenomenon more espe-  
cially when acid spinning baths are employed  
50 and particularly where zinc sulphate is present  
in the bath. Sulphuric acid is the acid generally  
used in such spinning baths.

Even if the deposit of material is insufficient to  
entirely clog the orifices, it acts to vary the thick-  
55 ness of the individual filaments, and consequently

produces undesirable properties in the final prod-  
uct. Also, so-called spinning hooks tend to form  
at the obstructions, either in or around the ori-  
fices of the spinneret, which, when filaments are  
extruded therethrough, might cause a temporary 5  
interruption of the spinning of a filament at the  
orifice affected, thus occasioning a tearing of the  
filament. These faults incur additional expense  
due to the manipulation necessary to change spin-  
nerets, the loss accruing from stopped produc- 10  
tion, and the increase in lower-quality yarns, for  
which yarns a lower price, only, may be asked.

The partial or total clogging of orifices is  
noticeable with the usual metal spinnerets, which  
spinnerets are made from gold, gold-palladium, 15  
gold-platinum, tantalum, et cetera. Furthermore,  
spinnerets are manufactured from precious  
and semi-precious stones, such as natural ruby,  
synthetic ruby, et cetera. Our improved pro-  
cedures are applicable in the use of these various 20  
types of spinnerets. The economic advantage of  
finding a simple, inexpensive method for keeping  
spinnerets operative during spinning is therefore  
apparent. As will be subsequently pointed out,  
other improved spinning conditions will be re- 25  
alized when following our procedures wherein we  
provide a solution for these problems in our pres-  
ent inventive concept.

Briefly, we have discovered that if certain cat-  
ion-active compounds are included either in the 30  
spinning bath and/or the spinning solution, the  
clogging of spinneret openings is considerably  
diminished or even prevented, and a very re-  
markable improvement of the spinning process  
per se will result. More specifically, cation- 35  
active aliphatic, carbocyclic or heterocyclic sub-  
stances have been employed with signal success in  
actual practice. By stating that "certain" cation-  
active compounds are employed it is intended to  
mean that only those cation-active compounds 40  
are suitable which are sufficiently soluble and sub-  
stantially stable in the spinning bath or the cel-  
lulosic solution or in both. Cation-active com-  
pounds are surface-active compounds which carry  
in the cation the group or radical which is re- 45  
sponsible for the surface activity. In contradis-  
tinction anion-active compounds are surface-  
active compounds which carry in the anion the  
group which is responsible for the surface ac-  
tivity. Such groups responsible for surface ac- 50  
tivity in this specification are called surface-  
active groups. Other groups or ions which are  
inert in this respect will be called surface-inac-  
tive or innocuous.

Surface activity as used herein is the property, 55

among other physico-chemical characteristics, of reducing surface or interfacial tension.

As an additional advantage we have found that when such cation-active substances are added to the viscose spinning bath, either by direct addition or as a result of addition to the viscose solution, the colloidal sulphur therein tends to agglomerate, and is easily filtered off if desired. Together with the removal of the sulphur thus effected, which in itself represents an impurity, other dissolved or suspended particles contaminating the spinning bath may be also precipitated and removed.

Surface activity depends upon the presence of one or more groups or radicals with long or extended chain-like structures which include extended aliphatic, carbocyclic and heterocyclic chains or combinations thereof. Compounds which contain a surface-active group show a tendency, according to the experiments and theory of Langmuir, to accumulate in the surface or interface of the solution and to assume an oriented position in which all of the extended chains lie parallel. Naturally, these substances can show this property only in so far as they are dissolved. When the molecules ionize, the surface activity may be induced by either the cation or the anion. This depends upon the position of the extended chain when the molecule ionizes. If, when the molecule ionizes, the extended chain remains with that part of the molecule bearing the positive charge, then it is said to be cation-active; whereas, on the other hand, if the long chain remains with that part of the molecule which bears a negative charge, it is said to be anion-active. Most of the usual surface-active substances are anion-active, with which substances the present invention is not concerned.

The compounds as exemplified below are illustrative of compounds which may be used in accordance with our invention. A general structural formula for a compound of this type may be expressed as



represents the cation and  $A^\circ$  represents the anion.  $X$  represents a polyvalent atom, or a radical containing such an atom, capable of being linked to a negative atom or radical and at the same time to one or more other atoms or radicals. The letter  $y$  indicates the valence of the atom or radical  $X$ . The invention also contemplates the presence of more than one atom symbolized by  $X$  in the cation. In this event one or more of the  $X$  atoms may be linked to surface-active groups and to surface-inactive atoms or radicals as described herein.  $S$  designates the radical or radicals inducing cation-activity, which are linked directly to the polyvalent atom of  $X$ .  $S$  may include one or more of the same or different aliphatic, carbocyclic and heterocyclic radicals and the letter  $m$  is a positive whole number indicating the total number of such radicals. The radical or radicals  $S$  should be such that when linked to  $X$  it or they will provide, in an ionizing solvent, a surface-active cation.  $R$  may be hydrogen and/or one or more of the same or different aliphatic, carbocyclic or heterocyclic radical or radi-

5

calls which are distinguished from those of  $S$  in that they do not induce surface-activity into the cation. The letter  $n$  is a positive whole number or zero and indicates the total number of such radicals and/or hydrogen atoms. This letter  $n$  also indicates the number of valences of the atom of  $X$  which remain available to be saturated by inactive atoms or radicals of the cation.

10

The letter  $A$  represents an innocuous anion, i. e., an anion having no surface-activity or at least less surface activity than the cation. This anion is linked directly to the polyvalent atom of  $X$  and may be an atom or an inorganic or organic radical. The letter  $c$  is a whole number indicating the valence of the anion. The letter  $C$  15 outside of the bracket is a whole positive number indicating the number of cations linked to the anion. In the examples given herein  $C$  equals  $c$  and the sum of  $n$  and  $m$  equals  $y-1$ .

20

It is to be understood that all compounds of the above named general structure have the character of bases (wherein  $A$  would be a hydroxyl radical) or their salts, including acid salts.

25

The more important cation-active compounds which may be employed in accordance with the present invention are the bases or their salts, such as may be derived from pentavalent nitrogen, and further the sulphonium, phosphonium and arsonium, etc. bases and their salts. The polyvalent atom of  $X$  in the foregoing formula is in 30 these compounds nitrogen, sulphur, phosphorus and arsenic, etc., respectively. The quaternary ammonium compounds are examples of compounds containing such an atom, nitrogen being the polyvalent atom. Of these, the pyridonium 35 or pyridinium compounds are examples of compounds in which the polyvalent atom, nitrogen, is contained in a radical, the radical being the pyridine ring ( $C_5H_5N$ ) having a valence of two. Other radicals containing the polyvalent atom 40 may, of course, be used in place of the pyridine ring.

45

In the bases or their salts illustrated by the above formula the innocuous anion symbolized by  $A$  is the hydroxide, chloride, sulphate, bromide, iodide, acetate, etc. The groups inducing cation activity symbolized by  $S_m$  comprise extended chain-like structures, such as aliphatic hydrocarbon chains having six or more carbon atoms therein. Also, the extended chain-like structures 50 may be composed of two or more benzene nuclei or other cyclic radicals, either combined directly or, for example, through a carbon or nitrogen or other linkages, with or without aliphatic chains substituted for the hydrogen in rings. 55

5

Referring now in detail to specific examples of suitable compounds, bases derived from nitrogen and their salts, for instance, certain pyridinium and other quaternary ammonium compounds, have been found to be particularly suitable. The 60 former compounds may include pyridinium bases or salts having linked thereto extended aliphatic chains, containing, for example, six or more carbon atoms and preferably 12 to 20 carbon atoms. Specifically, dodecyl, hexadecyl, octadecyl, or 65 even a lower carbon chain such as decyl may be linked to the nitrogen atom in the bases or salts of pyridinium such as pyridinium hydroxide, pyridinium sulphate or bisulphate and pyridinium bromide. Use may also be made of replacement 70 or substitute compounds such as the analogous substitution products of pyridine known as picoline ( $C_5H_4N(CH_3)$ ), and quinoline ( $C_9H_7N$ ), etc., and also compounds such as piperidine, acridine, cinnoline and naphthyridin and their derivatives. 75

An example of such compound is the bisulphate or acid sulphate of dodecyl-pyridinium, having the structure:



10 In this compound the letter  $X$  represents the pyridine radical



including the polyvalent atom nitrogen and having a valence  $y$  of 2; S is the dodecyl radical  $C_{12}H_{25}$  connected directly to the polyvalent atom (nitrogen) of  $X$ , the letter  $m$  being 1. The innocuous anion A is the bisulphate radical ( $HSO_4$ ) connected directly to the polyvalent atom of  $X$ . The valence of A is 1, and the letter C just outside the bracket is 1. In this compound the value of  $n$  is 0, so there would be no atom or radical R.

If the other hydrogen of the bisulphate were replaced by a second dodecyl pyridinium group the innocuous anion ( $SO_4$ ) would have a valence of 2 and the letter C outside the bracket would become 2, indicating two dodecyl pyridinium groups satisfying the two valences of the anion.

In the bases or salts of picoline and quinoline the ( $C_5H_4N(CH_3)$ ) and the ( $C_9H_7N$ ) groups, respectively, would be the radical  $X$  containing the polyvalent atom, nitrogen.

In the other quaternary ammonium compounds the same innocuous anions and surface-active groups may be linked to the pentavalent nitrogen atom as are employed with the pyridinium compounds. In this case  $X$  represents the atom nitrogen, having five valences. The three valences which are saturated in the pyridinium compounds by  $(CH_3)_5$  are now saturated by alkyl, aryl or other carbocyclic or heterocyclic groups and/or hydrogen atoms. For instance, three methyl groups may be used to form trimethyl dodecyl ammonium bromide. The following is the structural formula of such a compound:



55 In this case R would be the  $(CH_3)$  radical, the letter  $n$  being 3, and A would be the bromine atom.

If two butyl radicals are substituted for two of the methyl radicals in the above compound, methyl-dibutyl-dodecyl ammonium bromide would be formed. In this event the R would represent different radicals ( $CH_3$  and  $C_4H_9$ ), the total number of which would be 3.

Also the compound might contain more than one dodecyl radical or other radical capable of inducing the surface-activity of the cation. For example, one or more of the methyl radicals in the above compound might be replaced by a dodecyl radical, in which event the letter  $m$  would be 2 or more, depending upon how many methyl radicals were so replaced, and the letter  $n$  would be correspondingly decreased. If all the methyl radicals were replaced by radicals capable of inducing the surface activity of the cation, the letter  $n$  would, of course, become zero.

As previously indicated the radicals capable of inducing the surface-activity of the cation may include aromatic or other carbocyclic or heterocyclic radicals. The following compounds are examples of compounds containing such radicals including benzene nuclei in the surface-active groups in the cation: toluene azophenyl-trimethyl ammonium iodide, benzene azophenyl trimethyl ammonium iodide, diphenyl azophenyl trimethyl ammonium methyl sulphate, isopropyl naphthyl trimethyl ammonium iodide. In such compounds the



or



etc. represent the radicals inducing the surface-activity of the cation (S). These may be connected to a polyvalent atom as in the ammonium salts referred to or to the polyvalent element of a radical, as in the case of the pyridinium and similar compounds. It is obvious that both aliphatic radicals, for example, such as the dodecyl group, and carbocyclic or heterocyclic radicals, for example, such as the aromatic azo compounds referred to above, may be present in the compound as radicals inducing the surface activity of the cation.

Where the innocuous anion is divalent, as in the case of a sulphate in which both hydrogens are replaced by surface-active cations, a compound of the following type may be used:



40

di (dodecyl-triethyl ammonium) sulphate.

By the same token that the cation-active pyridinium and other ammonium compounds are suitable in connection with the present invention, sulphonium, phosphonium and arsonium bases and their salts may also be used. Of course, in order for this to be true, the sulphur, phosphorus or arsenic must have linked directly thereto, an innocuous anion and at least one group inducing surface activity in the cation. It is apparent that the sulphur being tetravalent, as distinguished from the pentavalent phosphorus and arsenic will have less valences to be saturated than in the case of phosphorus, arsenic and nitrogen. For example, a sulphonium compound such as d'ethyl dodecyl sulphonium hydroxide would correspond to triethyl dodecyl phosphonium hydroxide, either of which might be used. As further examples of these types of compounds, trimethyl dodecyl phosphonium hydroxide and dipropyl dodecyl sulphonium bromide may be employed.

It is also within the scope of our invention to use compounds in which the polyvalent atom of  $X$  is divalent or trivalent. The prerequisites of such an element must be that they will combine with an innocuous anion and a group inducing surface-activity in the cation.

The following are a number of compounds that may be used in accordance with our invention:

Octyl pyridinium iodide, dodecyl pyridinium bromide, hexadecyl pyridinium iodide, octadecyl pyridinium bromide, dodecyl pyridinium iodide, dodecyl pyridinium chloride, dodecyl-triethyl ammonium iodide, octyl-triethyl ammonium iodide,

75

decyl-triethyl ammonium iodide, dodecyl-triethyl ammonium iodide, hexadecyl-triethyl ammonium iodide, toluene azophenyl-trimethyl ammonium iodide, benzene azophenyl-trimethyl ammonium iodide, diphenyl-azophenyl-trimethyl ammonium methylsulphate, isopropyl-naphthyl-trimethyl ammonium iodide, diethyl-dodecyl sulphonium hydroxide, triethyl-dodecyl phosphonium hydroxide, trimethyl-dodecyl phosphonium iodide, trimethyl-dodecyl phosphonium bromide, dipropyl-dodecyl sulphonium bromide, etc.

Also unsaturated as well as saturated aliphatic radicals may be used as the radical inducing surface-activity in the cation (S) or as the inactive radical (R).

As pointed out above, the cation-active compounds may be added directly to the viscose spinning baths, or may be mixed with the viscose solution prior to extrusion into the baths, or they may be employed simultaneously in both the bath and spinning solution. It is of course necessary to select a cation-active compound which is not adversely affected by the acid of the bath and is substantially stable when used therein, and/or one that is stable in viscose when used therein. Compounds which are sufficiently soluble in dilute caustic soda or viscose to go into molecular solution in the viscose itself are particularly adapted to be added to the spinning solution. The tetra-alkylammonium bases and salts and aryltrialkylammonium bases and salts are especially suited for this purpose because of their greater stability toward the alkali of the viscose. When the compound is added to the spinning bath it is preferred to use a compound that goes into molecular solution in the spinning bath.

We herewith give three specific examples in order to more clearly disclose the present process:

*Example 1*

Ordinary viscose solution is made up, and spun or extruded through fine orifices in precious metal spinnerets into a well-known acid spinning bath, containing sulphuric acid, sodium sulphate, ammonium sulphate, and a small quantity of zinc sulphate. Such a bath, although widely known and used, is ordinarily troublesome since spinning difficulties due to the contaminated spinnerets, are common. We add to the bath, however, a small quantity (0.04 per cent by weight) of dodecyl pyridinium bisulphate. A desirable range of this material is between one thousandth per cent and eight hundredth per cent. Such a small addition eliminates most of the spinning irregularities and difficulties, and enables a much longer spinning time free from the noted interruptions than has been heretofore possible.

*Example 2*

An ordinary viscose solution is extruded through gold-palladium spinnerets into a spinning bath of the type mentioned in Example 1, but which contains a relatively larger amount of zinc sulphate, for example, five per cent of this salt. Ordinarily, under these conditions, the spinnerets become sufficiently contaminated in a few hours to deleteriously affect spinning, as pointed out above. However, if 0.1 per cent by weight of dodecyl triethyl ammonium iodide is first added to the viscose solution, the tendency to clog the holes of the spinnerets will be greatly reduced.

*Example 3*

An ordinary viscose solution is spun through gold-palladium spinnerets into a spinning bath

containing, for example, in addition to the usual bath ingredients 5% zinc sulphate; under these conditions the holes of the spinnerets will become contaminated within a few hours. If, however, 0.05% toluene azophenyl-trimethyl ammonium iodide is added to the viscose solution, there will be much less clogging of the spinneret holes.

We believe it remarkable that such small and relatively inexpensive amounts of substances may be employed, and still give such good results.

It must be understood that if the addition is made to the spinning bath rather than to the spinning solution, as set forth in Example 1, small further additions are necessary from time to time to replenish the compound lost or removed during the spinning operation.

By "yarn" we intend to cover filaments, threads, ribbons, foils, or other products usually produced by extrusion or spinning of a so-called cellulosic solution of artificial origin.

Having now set forth our invention as required by the patent statutes, we desire to be limited only to the extent set forth in the following claims.

What we claim is:

1. In the manufacture of yarn of artificial origin wherein a cellulosic solution is extruded through minute orifices into a coagulating medium to form filaments and the like therefrom, the step which comprises spinning the filaments in the presence of a dissolved cation-active ammonium compound having linked thereto an atomic grouping containing benzene nuclei inducing cation-activity and an innocuous anion.

2. A method as defined in claim 1 in which the atomic grouping includes a chain of benzene nuclei connected by an azo group.

3. In the manufacture of viscose yarn wherein the viscose solution is extruded through minute orifices into an acid precipitating bath to form filaments and the like therefrom, the step which comprises spinning the viscose filaments in the presence of a dissolved, cation-active, aryl substituted ammonium compound having an innocuous anion, said compound being substantially stable under spinning conditions.

4. A method as defined in claim 3 in which toluene azophenyl-trimethyl ammonium iodide is added to the viscose solution before extruding.

5. A method as defined in claim 3 in which about .05% toluene azophenyl-trimethyl ammonium iodide is added to the viscose solution before extruding.

6. A method as defined in claim 3 in which isopropyl-naphthyl-trimethyl-ammonium iodide is added to the viscose solution before extruding.

7. A method as defined in claim 3 in which benzene azophenyl-trimethyl-ammonium iodide is added to the viscose solution before extruding.

8. In the manufacture of cellulosic materials of artificial origin wherein a viscose solution is extruded through minute orifices into an acid precipitating bath to form filaments and the like therefrom, the step comprising spinning the filaments in the presence of a dissolved ammonium substituted cation-active compound containing an alkyl group and an aryl group and an innocuous anion.

9. In the manufacture of cellulosic materials wherein a viscose solution is extruded through minute orifices into an acid precipitating bath to form filaments and the like therefrom, the step which comprises extruding a viscose solution having dissolved therein an ammonium substi-

tuted cation-active compound containing an aryl group and an innocuous anion.

10. In the manufacture of cellulosic materials wherein a viscose solution is extruded through minute orifices into an acid precipitating bath to form filaments and the like therefrom, the step

which comprises extruding a viscose solution having dissolved therein an ammonium substituted cation-active compound containing an aryl group and an alkyl group and an innocuous anion.

JAMES J. POLAK.

JOHANNES G. WEELDENBURG.